

Oct. 16, 1928.

1,688,043

J. A. GANN

ALLOY

Filed Oct. 27, 1921



INVENTOR.

John A. Gann

BY

Day, Oberlin & Day

ATTORNEY

## UNITED STATES PATENT OFFICE.

JOHN A. GANN, OF MIDLAND, MICHIGAN, ASSIGNOR TO THE DOW CHEMICAL COMPANY,  
OF MIDLAND, MICHIGAN, A CORPORATION OF MICHIGAN.

## ALLOY.

Application filed October 27, 1921. Serial No. 510,797.

The present improved alloy is one in which magnesium is the predominant element, the object being to develop an alloy that will possess the characteristic lightness which is obtained by the use of magnesium in excess of 80 per cent, while such alloy will be characterized by high strength and high toughness and hardness sufficient for satisfactory use in the pistons of internal combustion engines for example. It is not intended, however, to limit the field of use in the mechanical arts to which an alloy possessing the lightness and physical characteristics of the one in hand may be applied. Primarily, the present improved alloy contains, in addition to magnesium in the predominant proportion indicated, aluminum and copper, thus constituting a ternary alloy. However, the characteristics of the alloy may be modified by the addition of further metals, specifically one or more of the following, viz, cadmium, tin and zinc, in relatively small amounts.

The present invention accordingly consists of such ternary alloy with or without the addition of such further metals, together with the steps involved in the making of such alloy hereinafter fully described and particularly pointed out in the claims. The annexed drawing and following description it will be understood set forth but one of several ways in which the invention may be carried out.

In said annexed drawing:—

The single figure there appearing is a diagrammatic representation of certain physical properties discovered in a typical ternary magnesium-aluminum-copper alloy of the class in hand, wherein the copper content remains constant while the aluminum content varies.

In such diagrammatic figure the physical properties represented, it will be noted, are the impact-toughness, hardness and tensile-strength, such impact-toughness being determined by the single-blow method and the hardness by the Brinell method and scaled to correspond with such impact-toughness. The curves in the diagram are not necessarily accurate representations throughout of the exact response of such alloy to tests of the character described, but do represent the manner in which the characteristic properties in question vary throughout the range under consideration which, as already indicated, includes not less than 80 per cent of magnesium, the balance being made up of aluminum

and copper with or without the addition in smaller amount of one or more of the following, viz, cadmium, tin and zinc.

For a ternary alloy that will be properly balanced with respect to the characteristics in question and at the same time have a sufficiently high thermal conductivity to adapt same for use in pistons in internal combustion motors, I prefer to use magnesium 90 per cent; aluminum 9 per cent and copper 1 per cent. Castings made from such alloy will have a specific gravity of approximately 1.80; tensile strength of approximately 17000 pounds per square inch; Brinell hardness of 52; and single-blow impact-toughness of 30.

For certain conditions of use, I find that the amount of the aluminum may be slightly reduced and cadmium, tin or zinc added, thus making a quarternary alloy. A satisfactory formula for this type will consist of magnesium 90 per cent; aluminum 8 per cent; copper 1 per cent and cadmium (or tin or zinc, as the case may be) 1 per cent.

As an alternative to reducing the relative proportion of aluminum, the amount of magnesium may be reduced and instead of adding but one additional ingredient, two metals, for example, cadmium and zinc, may be added with excellent results. The following is a formula for such a quinary alloy, viz, magnesium 87.85 per cent; aluminum 8.50 per cent; copper 2 per cent; cadmium 1 per cent and zinc 0.65 per cent.

To make my improved alloy, a measured quantity of pure magnesium metal is first melted in a suitable pot along with a proper amount of a flux that, while heavier than such metal, will have proper surface tension to promptly and effectively coat the metal.

As an example of such a flux, approximately equal parts of anhydrous magnesium chloride and sodium chloride may be employed, and if the specific gravity of such flux proves inadequate to float the metal after it has been alloyed, a small amount of barium chloride may be added. A small amount of the molten magnesium metal is then taken up in a ladle and the whole or part of the aluminum and copper, depending upon the total percentage thereof to be added to the batch, is placed in such ladle and melted with the magnesium therein, thereby producing an alloy relatively high in the alloying ingredients. The contents of the ladle are then gradually added to the main body of molten

- magnesium, (the operation being repeated until all of the alloying ingredients are added), with the result that the aluminum and copper forming such ingredients will diffuse throughout the mass and not drop through into the body of flux in which the latter floats and so be lost. As soon as the introduction of such alloying ingredients has been thus effected, the whole mass is well puddled and the operation may then be regarded as complete and the molten alloy cast either into ingots or directly into the form of mechanical parts, such as pistons or the like, for which it is intended to be used.
- 15 Where either cadmium, tin or zinc, or any two thereof, are to be added to the ternary alloy in accordance with formulas such as those hereinbefore set forth, the relatively small amount of such additional metal or 20 metals may be separately introduced in the same fashion as the two entering into the ternary alloy, or they may be at once added along with such two in forming the preliminary alloy which is subsequently added to the 25 main body of the molten magnesium metal, resulting in the production of an alloy in which such magnesium is the predominant ingredient. On the other hand, in some cases such additional ingredients may be conveniently combined with each other before being 30 thus alloyed with magnesium, the final result of course being the same.
- Other modes of applying the principle of my invention may be employed instead of the 35 one explained, change being made as regards the steps herein disclosed or the ingredients employed in carrying out such steps, pro-

vided the steps or ingredients set forth in the following claims or the equivalent of such steps or ingredients be employed.

40

I therefore particularly point out and distinctly claim as my invention:—

1. As a new product, an alloy containing approximately ninety per cent of magnesium, nine per cent of aluminum, and less than one and one-half per cent of copper.

45

2. As a new product, an alloy containing approximately ninety per cent of magnesium, nine per cent of aluminum, and copper, cadmium and zinc each in small but consequential percentages.

50

3. The method of making a magnesium-aluminum-copper alloy, wherein the magnesium largely predominates, which consists in first interfusing the desired amount of aluminum and the desired amount of copper with a relatively small quantity of the total magnesium in such alloy, and then adding the resulting alloy to the remaining quantity of magnesium in molten state.

55

4. The method of making a magnesium-aluminum-copper alloy, wherein the magnesium largely predominates, which consists in first interfusing the desired amount of aluminum and the desired amount of copper with a relatively small quantity of the total magnesium in such alloy, whereby an alloy relatively high in aluminum and copper is produced, and then adding such resulting alloy to the remaining quantity of magnesium.

60

Signed by me this 24th day of October, 1921.

JOHN A. GANN.

70